# EUROPEAN PATENT SPECIFICATION

(11) **EP 2 152 528 B1**
(45) Date of publication and mention of the grant of the patent: **05.03.2014**
(21) Application number: 08766715.0
(22) Date of filing: 30.05.2008
(51) Int. Cl.: B44C 5/04

(54) **METHOD FOR MANUFACTURING A DECORATIVE PANEL AND A DECORATIVE PANEL**
VERFAHREN ZUR HERSTELLUNG EINER ZIERPLATTE UND ZIERPLATTE
PANNEAU DÉCORATIF ET SON PROCÉDÉ DE FABRICATION

(30) Priority: 01.06.2007 NL 1033924
(43) Date of publication of application: 17.02.2010
(73) Proprietor: Trespa International B.V., 6002 SM Weert (NL)
(72) Inventor: VAN DE WALL, WILHELMUS Josephus Alex, 5591 CS Heeze (NL); VOGELS-JANSEN, Irma, 6021 ZS Budel (NL)
(74) Representative: Algemeen Octrooi- en Merkenbureau B.V.
(86) International application number: PCT/NL2008/000142
(87) International publication number: WO 2008/147180

(56) References cited:
- EP-A- 0 216 269
- EP-A- 0 338 221
- EP-A- 0 706 834
- EP-A- 1 319 524
- EP-A- 1 470 933
- WO-A-00/22039
- WO-A-00/44576
- WO-A-2005/009758
- DE-A- 3 418 282
- DE-A- 3 533 737
- DE-A- 19 842 510
- US-A- 4 789 604

## Description

The present invention relates to a method for manufacturing a decorative panel for exterior use, in which a core and a decorative layer, which decorative layer comprises radiation-curable components, are placed in a press and are pressed together therein under elevated temperature and pressure conditions. The present invention further relates to a decorative panel comprising a core provided with a decorative layer, which decorative layer comprises a radiation-curable component.

From German Offenlegungsschrift DE 34 18 282 there is known a method for manufacturing a decorative panel, wherein a decorative layer is applied to an underlay, which decorative layer comprises a mixture of radiation-polymerisable components, after which the decorative layer is irradiated and pressed together with the underlay to obtain a scratch resistance of at least about 1.5 Newton.

From International application WO 00/22039 there is known a method for manufacturing a laminate, in which a planar substrate is provided with a coating based on acrylate polymers, to which coating SiO₂ nanoparticles have been added to give the laminate material a scratch resistance of at least 3.5 Newton. Such materials are in particular used for floors, in which application scratch resistance is an important parameter.

From U.S. Pat. No. 4,789,604 in the name of the present applicant there is known a method for manufacturing a decorative panel, in which a liquid synthetic resin layer is a applied to a substrate layer, after which a film having a surface roughness is applied to the resin layer, said surface roughness being transferred to the resin layer, after which the resin layer is polymerised by exposure to radiation. Subsequently, the resin layer and the substrate are pressed together under elevated temperature conditions.

From European patent application No. 0 338 221 there is known a radiation-curable coating, to which coating, which is based on an acrylate mixture, matting agents are added in an amount of 20 - 60 weight percentage. Setting the matting degree by means of matting agents has appeared to be difficult in practice, because the matting agents adversely affect the crosslinking reaction of the matrix material, whilst in addition the use of matting agents has an adverse effect on the scratch resistance of a coating thus obtained.

From European patent application No. 0 706 834 there is known a method for producing a substrate material provided with a UV curable lacquer consisting of a lacquer based on an acrylate mixture, a UV initiator and other usual additives. The matting degree of the aforesaid UV lacquer is adjusted by the addition of mono- and/or di-functional monomers, and UV hardening is effected with several radiation sources with a defined range of wavelengths. Thus a first UV source is used which emits monochromatic UV in the range 100-200 nm, whereupon the coating thus applied to the substrate layer is subjected to a second radiation stage, using UV radiation having a higher a wavelength.

From German Offenlegungsschrift DE 198 42 510 there is known a method for structuring the surface of a UV curable lacquer, using UV radiation having a wavelength of maximally 250 nm. Subsequently, a postouring treatment with long-wave UV or EB (electron beam) radiation must take place. An example of a UV curable lacquer mentioned therein is a mixture of monomers and prepolymers of acrylate components, using paper or a plastic in a thickness of 80-500 µm as the substrate material.

European patent application 1 470 933 relates to a method for the produotion of sheet materials with a varnish-containing protective layer obtained by coating a carrier material with varnlah, hardening the varnish, combining the varnished side of the coated carrier with the sheet material and then removing the carrier, using a varnish containing radically- and/or ionically-polymerisable substances, which is at least partly hardened on the carrier by radical and/or ionic polymerization.

International application WO 2005/009758 relates to method for producing a sheet-like or web-like, decorative, scratch- and/or abrasion-resistant coating material, comprising the steps: coating a support layer with a liquid or pasty base layer comprising radiation-curing resins but no heat-curing resins and also an abrasive filler, drying the support layer thus coated by supplying heat, applying a covering layer to the dried base layer, and jointly curing and/or crosslinking the covering layer and also the radiation-curing resins in the base layer by irradiating the covering layer with UV and/or electron beams.

The traditional process of manufacturing HPL (high-pressure laminates) and HPL compact plates is carried out in a press under elevated temperature and pressure conditions. The melamine resin that is used will melt under said elevated temperature conditions in the press member and subsequently liquefy, with the surface of the melamine resin more or less taking on the microstructure of the press. The thus structured melamine resin will form a highly crosslinked network as a result of the elevated temperature conditions and form a scratch-resistant and hard coating after being removed from the press.

The present inventors have found that obtaining a microstructure In radiation-curable surfaces is possible only to a limited degree, because the degree of gloss will Increase again after some time, which effect occurs In particular In the case of exterior use. The present inventors attribute such a change in the degree of gloss to the stress relaxation In the thermosetting coating.

The object of the present invention is thus to provide a method for manufacturing a decorative panel, in which a decorative layer comprising radiation-curable components is used, which decorative layer can be given a structure that will be retained for a prolonged period of time.

Another object of the present invention is to provide a method for manufacturing a decorative panel, in which the decorative layer comprises radiation-curable components, which decorative layer can be given a structure which will remain stable for a prolonged period of time even after being exposed to moisture and temperature and environmental influences, and which will not lead to visually unacceptable changes in gloss.

The method as referred to in the introduction is characterised in that before the pressing operation, the decorative layer is subjected to a radiation treatment comprising a first radiation stage, using a wavelength in the 100-250 nm range, and a second radiation stage, using long-wave UV and/or electron beam (EB) radiation, so as to minimise the change in the degree of gloss in the thus cured decorative layer.

The present inventors have surprisingly found that the degree of gloss thus obtained is retained for a prolonged period of time when the aforesaid radiation treatment is carried out first and subsequently the pressing operation. After the decorative layer has been subjected to a radiation treatment, using a wavelength in the 100-250 nm range, it is preferable to carry out a post-curing step, using long-wave UV radiation, viz. a wavelength in the 200-400 nm range, or EB (electron beam) radiation. The present inventors assume that the decorative layer will exhibit a slightly matted surface as a result of the aforesaid radiation treatment comprising two radiation stages, after which the surface will plasticize or deform during the pressing operation under elevated temperature conditions and there will no longer be any stress relaxation after the pressing operation, so that the thus obtained degree of gloss will be practically stable from the viewpoint of time. The structured surface of the press member will thus be incorporated in the decorative layer practically in a substantially stress-free and reversible manner. Preferably, the decorative layer does not comprise any solid particles, the decorative layer in particular comprises maximally 5%, more in particular maximally 1% solid particles, notably amorphous SiO₂ nanoparticles, based on the weight of the cured decorative layer.

Suitable radiation-curable components include (meth)acrylate compounds, for example epoxy (meth)acrylate, silicone (meth)acrylate, polyester (meth)acrylate and urethane (meth)acrylate. The decorative layer may also comprise mono(meth)acrylate, di(meth)acrylate, tri(meth)acrylate, tetra(meth)acrylate, penta(meth)acrylate and hexa(meth)acrylate. The core layer is in principle not critical and may comprise a material selected from the group consisting of wood, a number of paper layers, plastics, metals, nonwovens and fibre mats, which may or may not be impregnated with a resin.

In a special embodiment of the present invention, the decorative layer comprises an underlayer, which underlayer comprises paper, and which underlayer is present on a core layer comprising a stack of fibre-containing layers, wherein the underlayer and the decorative layer present thereon is supported on the fibre-containing layers during the pressing operation, such that the radiation-cured decorative layer forms the outermost layer of the decorative panel. The paper used for the underlayer may contain partially cured thermosetting synthetic resins.

The stack of fibre-containing layers is preferably selected from the group consisting of sodium kraft paper, a bound fabric and a densified fibre mat, which bound fabric is preferably selected from the group consisting of wood and cellulose fibres, wherein the pressing operation is carried out at a temperature of about 80-220 °C, in particular 120-220 °C, and a pressure of about 500-10.000 kPa (5-100 bar), in particular 1000-10.000 kPa (10-100 bar).

The first radiation treatment of the decorative layer, during which matting takes place, is carried out at a wavelength in the 100-250 nm range, preferably in the 170-230 nm range, in particular 170-180 nm, in particular using a radiation source which emits monochromatic radiation having a wavelength of 172 nm. In specific embodiments it is preferable to use a radiation source which emits monochromatic radiation having a wavelength of 222 nm. The total radiation dose preferably ranges between 1-300 mJ/m², preferably between 3-12 mJ/m². After the first radiation treatment a second radiation treatment, viz. full curing with long-wave UV or EB radiation, is preferably carried out.

It is in particular preferable if a press member having a structured surface is used during said pressing operation, which structured surface in particular abuts against the radiation-curable layer so as to thus transfer the structure of the pressure plate to the radiation-curabte layer.

The present invention further relates to a decorative panel comprising a core provided with a decorative layer having a structured surface, which decorative layer comprises a radiation-curable component, characterised by the characterizing portion of claim 12. It is in particular preferable if the degree of gloss changes by no more than 50%, tested according to EN438-2:2005, part 29 in an exterior application.

It has been found to be possible, using the present method, to manufacture a decorative panel whose degree of gloss changes by maximally 10 units, measured at an angle of 60° and tested for 3000 hours according to EN438-2:2005, part 29.

The present invention in particular concerns the pre-matting of the radiation-curable layer, thereby giving the radiation-curable layer a so-called matted surface, after which the assembly of core and decorative layer is placed in a press, in which the decorative layer will plasticize to some extent as a result of the elevated temperature conditions therein, as a result of which the structure of the press member is "frozen" into the decorative layer without any stress relaxation taking place. A decorative panel manufactured in this way will exhibit a degree of gloss that will remain stable for a prolonged period of time.

The invention therefore relates to the use of a radiation treatment comprising a first radiation stage, using a wavelength in the 100-250 nm range, and a second radiation stage, using long-wave UV and/or electron beam (EB) radiation, so as to minimise the change in the degree of gloss in a decorative layer having a structured surface comprising radiation-curable components. Because of the special use of the present decorative panel in exterior environments, especially the degree of gloss, in particular the change therein, is an important and critical parameter.

The present application will be explained hereinafter by means of a number of examples and associated figures 1-4, in which connection it should be noted, however, that the present invention is by no means limited to such special examples.
Figures 1-4 show recordings of panel surfaces.

### Comparative Example 1

A panel was used which consisted of a core of cellulose-containing fibre mats impregnated with phenol resol resin, which core was provided on either side thereof with a substrate layer consisting of a paper impregnated with phenol resol resin, which substrate layer was subsequently provided with a decorative layer comprising two pigmented or unpigmented radiation-curable (cured by means of EB radiation) layers, the outermost layer of the panel being a transparent layer consisting of transparent; acrylate-containing polyester urethane oligomers dissolved in 35% hexane diol diacrylate.

The above-described panel was compressed for a period of about 25 minutes at a temperature of about 165 °C, using a pressure of 6,5 MPa (65 bar), so as to obtain a rigid panel. The aforesaid pressing operation was carried out by means of a press member, viz. a pressure plate having a coarse structure. After the pressing operation, the degree of gloss was 40 units, measured at an angle of 60°. The aforesaid value was indicated as glossy. After exposure of said panel to weather conditions for 67 hours, the degree of gloss increased by 10 to 20 units.

### Comparative Example 2

A panel similar to the panel described in Comparative Example 1 was compressed, but in this embodiment a pressure plate having a fine structure was used. After the pressure treatment, the degree of gloss was 20 units, measured at an angle of 60°. After exposure of said panel to the same weather conditions as in Comparative Example 1 for 67 hours, the degree of gloss increased by 30 to 40 units, measured at an angle of 60°. Figure 1 shows a recording of the surface structure directly after the pressure treatment, whilst figure 2 shows a recording made after the surface had been exposed to weather conditions for 67 hours.

### Example 3 (according to the present invention)

A panel similar to the panel used in Comparative Example 1 was used, except that, prior to the pressure operation, the decorative layer was first subjected to a radiation treatment, using a wavelength of 172 nm, with the total radiation dose being 10 mJ/m². The entire decorative layer was then subjected to a second radiation treatment, using EB radiation. After the surface had thus been matted and subsequently post-cured, a pressing operation was carried out under the conditions mentioned in Comparative Example 1, using a pressure plate having a coarse structure, as in Comparative Example 1. After the pressing operation, the degree of gloss of the thus obtained panel was 8 units, measured at an angle of 60°. After exposure to the same weather conditions as mentioned in Comparative Example 1 and Comparative Example 2 for more than 330 hours, the degree of gloss decreased by 2 to 3 unis, measured at an angle of 60°.

Figure 3 shows a recording of the surface directly after the pressing operation, whilst figure 4 shows a recording of the same surface, in this embodiment after exposure to weather conditions for 330 hours, however. Figures 3 and 4 clearly show that the macrostructure of the press member that was used partially disappears and that the matting of the surface, obtained by matting the decorative layer through radiation, remains visible.

The weather conditions as mentioned before for each of the comparative examples and for the example according to the present invention were:
- Light intensity: 0.55 W/m² at 340 nm, approx. 63 W/m² at 300-400 nm
- Air temperature: 50 °C
- Black panel
   temperature: 75 °C
- Cycle simulation: 120 minutes, of which 90 minutes light at an RH of 50 ± 2%, followed by 30 minutes exposure and sprinkling.

### Example 4: Test for exterior use, carried out according to EN438-2:2005, part 29

| Experiment | Exposure | Gloss after pressing, before testing measured at 60° | Gloss after 3000 hours of testing measured at 60° | Gloss after pressing, before testing measured at 85° | Gloss after 3000 hours of testing measured at 85° |
|---|---|---|---|---|---|
| A | none | 14.4 | 27.4 | 21.9 | 34.5 |
| B | 172 nm, followed by EB | 5.6 | 3.9 | 8,5 | 5.3 |

### Example 5: Test for exterior use

| | |
|---|---|
| Light intensity: | 0.55 W/m² at 340 nm is approx. 63 W/m² at 300-400 nm |
| air temperature: | 50 °C |
| Black panel temperature: | 75 °C |
| Cycle simulation: | 120 minute cycle, of which 90 minutes light at an RH of 50 +/- 2%, followed by 30 minutes exposure and sprinkling. |

| Experiment | Exposure | Gloss after pressing, before testing measured at 60° | Gloss after 2000 hours of testing measured at 60° | Gloss after pressing, before testing measured at 85° | Gloss after 2000 hours of testing measured at 85° |
|---|---|---|---|---|---|
| C | none | 14.4 | 27.9 | 21.9 | 36.2 |
| D | 172 nm, followed by EB | 5.6 | 3.8 | 8.5 | 5.1 |

### Example 6: Test for interior use

| | |
|---|---|
| Lamps: | UV-A 351 nm |
| Air temperature: | 60 +/- 3 °C |

Relative air humidity not controlled, depends on environment.

Normal test duration is discoloration from wool scale 6 to 5, this is 48 hours of testing.

| Experiment | Exposure | Gloss after pressing, before testing measured at 60° | Gloss after 3000 hours of testing measured at 60° | Gloss after pressing, before testing measured at 85° | Gloss after 66 hours of testing measured at 85° |
|---|---|---|---|---|---|
| E | none | 14.8 | 17.3 | 21.3 | 25.2 |
| F | 172 nm, followed by EB | 6.7 | 6 | 10.4 | 9.3 |

In examples 4-6 the panels A-F are similar to the panel described in Comparative Example 1.

## Claims

1. A method for manufacturing a decorative panel for exterior use, in which a core and a decorative layer, which decorative layer comprises radiation-curable components, are placed in a press and are pressed together therein under elevated temperature and pressure conditions so as to obtain the decorative panel, which press is provided with a structured surface, which structured surface abuts against the decorative layer during the pressing operation, **characterised in that** before the pressing operation, the decorative layer is subjected to a radiation treatment comprising a first radiation stage, using a wavelength in the 100-250 nm range, and a second radiation stage, using long-wave UV and/or electron beam (EB) radiation, so as to minimise the change in the degree of gloss in the thus cured decorative layer.

2. A method according to claim 1, **characterised in that** a wavelength in the 170-180 nm range is used for the first radiation stage.

3. A method according to claim 2, **characterised in that** a wavelength of 172 nm is used for the first radiation stage.

4. A method according to any one or more of claims 1-3, **characterised in that** a total radiation dose of 1-300 mJ/m² is used for the first radiation stage.

5. A method according to claim 4, **characterised in that** a total radiation dose of 3-12 mJ/m² is used for the first radiation stage.

6. A method according to any one or more of the preceding claims, **characterised in that** the decorative layer comprises an underlayer, which underlayer comprises paper, and which underlayer is present on the core comprising a stack of fibre-containing layers, wherein the underlayer and the decorative layer present thereon is supported on then fibre-containing layers during the pressing operation, such that the radiation-cured decorative layer forms the outermost layer of the decorative panel.

7. A method according to claim 6, **characterised in that** the stack of fibre-containing layers is selected from the group consisting of sodium kraft paper, a bound fabric and a densified fibre mat.

8. A method according to claim 7, **characterised in that** said bound fabric is selected from the group consisting of wood and cellulose fibres.

9. A method according to any one or more of the preceding claims, **characterised in that** the pressing operation is carried out at a temperature of about 80-220 °C and a pressure of about 500-10.000 kPa (5-100 bar).

10. A method according to claim 9, **characterised in that** the temperature ranges between 120 and 220 °C and the pressure ranges between 1000-10.000 kPa (10 and 100 bar).

11. A method according to any one or more of the preceding claims, **characterised in that** the decorative layer in particular comprises maximally 5%, in particular maximally 1% solid particles, notably amorphous SiO₂ nanoparticles, based on the weight of the cured decorative layer.

12. A decorative panel comprising a core provided with a decorative layer having a structured surface, which decorative layer comprises a radiation-curable component, **characterised in that** the degree of gloss is maximally 15, measured at an angle of 60° according to ASTM D523, wherein the degree of gloss changes by maximally 10 units, measured at an angle of 60° and tested for 3000 hours according to EN438-2:2005, part 29, in an exterior application.

13. A decorative panel according to claim 12, **characterised in that** the degree of gloss changes by no more than 50%, tested according to EN438-2:2005, part 29, in an exterior application.

14. Use of a radiation treatment comprising a first radiation stage, using a wavelength in the 100-250 nm range, and a second radiation stage, using long-wave UV and/or electron beam (EB) radiation, so as to minimise the change in the degree of gloss in a method for manufacturing a decorative layer on a decorative panel for exterior use having a structured surface comprising radiation-curable components.

## Patentansprüche

1. Verfahren zur Herstellung einer Zierplatte für den Außeneinsatz, wobei ein Kern und eine Zierschicht, die strahlungshärtbare Komponenten aufweist, in eine Presse gelegt werden und darin unter hohen Temperaturen und Druckbedingungen derart zusammengepresst werden, dass die Zierplatte erhalten wird, wobei die Presse mit einer strukturierten Oberfläche versehen ist, die während des Pressens an die Zierschicht angrenzt, **dadurch gekennzeichnet, dass** die Zierschicht vor dem Pressen einer Bestrahlung unterzogen wird, die eine erste Bestrahlungsstufe, die eine Wellenlänge im Bereich von 100-250 nm verwendet, und eine zweite Bestrahlungsstufe umfasst, die langwellige UV-und/oder Elektronenstrahlen-Strahlung verwendet, um die Änderung des Glanzgrads in der so gehärteten Zierschicht zu minimieren.

2. Verfahren nach Anspruch 1, **dadurch gekennzeichnet, dass** eine Wellenlänge im Bereich von 170-180 nm für die erste Bestrahlungsstufe verwendet wird.

3. Verfahren nach Anspruch 2, **dadurch gekennzeichnet, dass** eine Wellenlänge von 172 nm für die erste Bestrahlungsstufe verwendet wird.

4. Verfahren nach einem oder mehreren der Ansprüche 1 bis 3, **dadurch gekennzeichnet, dass** eine Gesamtstrahlungsdosis von 1-300 mJ/m² für die erste Bestrahlungsstufe verwendet wird.

5. Verfahren nach Anspruch 4, **dadurch gekennzeichnet, dass** eine Gesamtstrahlungsdosis von 3-12 mJ/m² für die erste Strahlungsstufe verwendet wird.

6. Verfahren nach einem oder mehreren der vorhergehenden Ansprüche, **dadurch gekennzeichnet, dass** die Zierschicht eine Unterschicht umfasst, die ein Papier aufweist, wobei das Papier auf dem Kern vorhanden ist, der einen Stapel aus faserenthaltenden Schichten umfasst, wobei die Unterschicht und die darauf vorhandende Zierschicht während des Pressens auf den faserenthaltenden Schichten derart gestützt werden, dass die strahlungsgehärtete Zierschicht die äußerste Schicht der Zierplatte ausbildet.

7. Verfahren nach Anspruch 6, **dadurch gekennzeichnet, dass** der Stapel aus faserenthaltenden Schichten aus der aus Natronkraftpapier, einem gebundenen Stoff und einer verdichteten Fasermatte bestehenden Gruppe ausgewählt ist.

8. Verfahren nach Anspruch 7, **dadurch gekennzeichnet, dass** der gebundene Stoff aus der aus Holz und Zellulosefasern bestehenden Gruppe ausgewählt ist.

9. Verfahren nach einem oder mehreren der vorhergehenden Ansprüche, **dadurch gekennzeichnet, dass** das Pressen bei einer Temperatur von etwa 80-220 °C und einem Druck von etwa 500-10.000 kPa (5-100 bar) ausgeführt wird.

10. Verfahren nach Anspruch 9, **dadurch gekennzeichnet, dass** sich die Temperatur im Bereich von 120 bis 220 °C und der Druck im Bereich von 1000 bis 10.000 kPa (10 bis 100 bar) liegt.

11. Verfahren nach einem oder mehreren der vorhergehenden Ansprüche, **dadurch gekennzeichnet, dass** die Zierschicht, mit Bezug auf das Gewicht der gehärteten Zierschicht, insbesondere maximal 5%, speziell maximal 1%, feste Partikel umfasst, insbesondere amorphe SiO₂-Nanopartikel.

12. Zierplatte mit einem Kern, der mit einer eine strukturierte Oberfläche aufweisenden Zierschicht versehen ist, die eine strahlungshärtbare Komponente aufweist, **dadurch gekennzeichnet, dass** der unter einem Winkel von 60° gemäß ASTM D523 gemessene Glanzgrad maximal 15 beträgt, wobei sich der unter einem Winkel von 60° gemessene und über 3000 Stunden nach EN438-2:2005, Teil 29 getestete Glanzgrad bei einem Außeneinsatz maximal um 10 Einheiten verändert.

13. Zierplatte nach Anspruch 12, **dadurch gekennzeichnet, dass** sich der nach EN438-2:2005, Teil 29 getestete Glanzgrad um nicht mehr als 50% bei einem Außeneinsatz verändert.

14. Verwendung einer Bestrahlung mit einer ersten Bestrahlungsstufe, die eine Wellenlänge im Bereich 100-250 nm verwendet, und einer zweiten Bestrahlungsstufe, die langwellige UV- und/oder Elektronenstrahlen-Strahlung verwendet, um die Änderung des Glanzgrads in einem Verfahren zur Herstellung einer eine strukturierte Oberfläche aufweisenden Zierschicht auf einer Zierplatte für den Außeneinsatz zu minimieren, wobei die Zierschicht strahlungshärtbare Komponenten aufweist.

## Revendications

1. Procédé de fabrication d'un panneau décoratif pour une utilisation extérieure, dans lequel une âme et une couche décorative, laquelle couche décorative comprend des composants durcissables par rayonnement, sont placées dans une presse et sont pressées ensemble dans celle-ci dans des conditions de température et de pression élevées de façon à obtenir le panneau décoratif, laquelle presse est dotée d'une surface structurée, laquelle surface structurée butte contre la couche décorative pendant l'opération de pressage, **caractérisé en ce qu'**avant l'opération de pressage, la couche décorative est soumise à un traitement de rayonnement comprenant une première étape de rayonnement, en utilisant une longueur d'onde dans la plage de 100 à 250 nm, et une seconde étape de rayonnement, en utilisant des UV à longues ondes et/ou un rayonnement de faisceaux d'électrons (FE), de façon à minimiser le changement de degré de brillant dans la couche décorative ainsi durcie.

2. Procédé selon la revendication 1, **caractérisé en ce qu'**une longueur d'onde dans la plage de 170 à 180 nm est utilisée pour la première étape de rayonnement.

3. Procédé selon la revendication 2, **caractérisé en ce qu'**une longueur d'onde de 172 nm est utilisée pour la première étape de rayonnement.

4. Procédé selon l'une quelconque ou plusieurs des revendications 1 à 3, **caractérisé en ce qu'**une dose de rayonnement total de 1 à 300 mJ/m² est utilisée pour la première étape de rayonnement.

5. Procédé selon la revendication 4, **caractérisé en ce qu'**une dose de rayonnement total de 3 à 12 mJ/m² est utilisée pour la première étape de rayonnement.

6. Procédé selon l'une quelconque ou plusieurs des revendications précédentes, **caractérisée en ce que** la couche décorative comprend une sous-couche, laquelle sous-couche comprend du papier, et laquelle sous-couche est présente sur l'âme comprenant un empilement de couches contenant des fibres, dans lequel la sous-couche et la couche décorative présente sur celle-ci sont supportées sur les couches contenant des fibres pendant l'opération de pressage, de sorte que la couche décorative durcie par rayonnement forme la couche la plus à l'extérieur du panneau décoratif.

7. Procédé selon la revendication 6, **caractérisé en ce que** l'empilement de couches contenant des fibres est choisi dans le groupe consistant en du papier kraft de sodium, une étoffe liée et un tapis de fibres densifiées.

8. Procédé selon la revendication 7, **caractérisé en ce que** ladite étoffe liée est choisie dans le groupe consistant en les fibres de bois et de cellulose.

9. Procédé selon l'une quelconque ou plusieurs des revendications précédentes, **caractérisé en ce que** l'opération de pressage est réalisée à une température d'environ 80 à 220 °C et une pression d'environ 500 à 10 000 kPa (5 à 100 bars).

10. Procédé selon la revendication 9, **caractérisé en ce que** la température est entre 120 et 220 °C et la pression est entre 1 000 et 10 000 kPa (10 et 100 bars).

11. Procédé selon l'une quelconque ou plusieurs des revendications précédentes, **caractérisé en ce que** la couche décorative comprend en particulier au maximum 5 %, en particulier au maximum 1 % de particules solides, notamment des nanoparticules de SiO₂ amorphe sur la base du poids de la couche décorative durcie.

12. Panneau décoratif comprenant une âme dotée d'une couche décorative ayant une surface structurée, laquelle couche décorative comprend un composant durcissable par rayonnement, **caractérisé en ce que** le degré de brillant est au maximum de 15, mesuré à un angle de 60 °C selon la norme ASTM D523, dans lequel
le degré de brillant change au maximum de 10 unités, mesuré à un angle de 60° et mis à l'essai pendant 3 000 heures selon la norme EN438-2-2005, partie 29, dans une application extérieure.

13. Panneau décoratif selon la revendication 12, **caractérisé en ce que** le degré de brillant change de pas plus de 50 %, mis à l'essai selon la norme EN438-2-2005, partie 29, dans une application extérieure.

14. Utilisation d'un traitement par rayonnement comprenant une première étape de rayonnement, en utilisant une longueur d'onde dans la plage de 100 à 250 nm, et une seconde étape de rayonnement, en utilisant des UV à longues ondes et/ou un rayonnement de faisceaux d'électrons (FE), de façon à minimiser le changement de degré de brillant dans un procédé de fabrication d'une couche décorative sur un panneau décoratif pour une utilisation extérieure ayant une surface structurée comprenant des éléments durcissables par rayonnement.
